

## UNITED STATES PATENT OFFICE

1,929,432

## METHOD OF MAKING PAPER AND SIMILAR PRODUCTS

Mone R. Isaacs, Philadelphia, Pa.

No Drawing. Application May 16, 1931, Serial No. 538,001. Renewed November 22, 1932

12 Claims. (Cl. 92—21)

My invention relates to the making of paper, cardboard and similar products made, in the main from a pulp of cellulose or similar fibers, and more particularly to the addition to the pulp of a binding material composed in the main of casein and a solvent therefor, for the purpose of imparting strength and the property of repelling moisture.

I have discovered that a better, stronger, more readily foldable and more waterproof paper, cardboard or the like may be produced by adding to the paper pulp in the beater, a binding composition composed of an animal or vegetable proteid or a mixture of the same, mixed or associated with lime and a fluoride and incorporating the same into and impregnating the fibers with this binder during the beating operation of the pulp.

The proteid which I have found to be the best suited for the purposes above stated, is casein, and it is to be understood that I prefer to use casein as the main or principal proteid in the binding composition for the cellulose fibers of the pulp, but other proteids, such as glue, starches, corn meal, tapioca meal or soya-bean meal may be used in minor quantities with the casein, for the purpose of reducing the cost of manufacture when the uses, to which the final products (paper, board or the like) are to be put, do not require the same high degree of water resistiveness or the degree of hardness which may be attained by the use of casein alone as the proteid of the composition.

These ingredients may be added to the cellulose fibers and the liquor therefor, comprising the pulp in the beater and before the beating operation is actually commenced or after the fibers have been beaten into a pulp of suitable consistency, and the ingredients may be added simultaneously as a binding composition mixed together with or without an admixture of water therewith, or there may be added separately and/or at different times during the beating operation.

The proportions of these ingredients which I add to each 100 pounds of pulp in the beater are substantially as follows:

Casein or a mixture of casein with other proteids, from 2 to 6 pounds to each 100 pounds of pulp;

Lime from 10% to 20% of the weight of the casein;

Sodium fluoride from 5% to 8% of the weight of the casein.

But I do not wish to be construed as limited

to the exact proportions above given, particularly with respect to the proportion of the binder to the pulp, for that may vary considerably, depending upon the quality of the paper or board being made. Generally speaking, the harder the product is to be, the greater will be the proportion of the binder.

I preferably mix these ingredients in the dry state, and when I wish to use the same to form a binder for pulp, I preferably add thereto a suitable amount of water to bring the mixture to the consistency of a paste or cream prior to its introduction into the pulp. They may, however, be added to the pulp in a dry state and in substantially any order or sequence. I prefer to add this binding material to the pulp after the beating of the pulp had been well started and near the end of the beating operation. If the ingredients are added separately it may be in any order, or the fluoride may be mixed with the lime, mixed with water or dry, and added to the pulp in the beater.

Lime, either quick lime or hydrated lime, has the property of rendering casein readily soluble in water, but I have discovered that a comparatively small quantity or proportion of lime is all that is necessary for the purpose of forming a binder for a cellulose pulp. Very much less lime is required than in the production of a paint or a coating material.

By thus impregnating the cellulose or other fibers of the pulp with a composition of casein, a small quantity of lime and a small quantity of a fluoride, such as sodium fluoride or other equivalents, I am able in the manufacture of paper to increase the strength of the paper made therefrom nearly 100%.

Thus a paper made with the ordinary binding materials usually employed, may have, for example, a "pop" test strength of 33 on a Mullen testing machine. With the same pulp stock and by substituting my improved binder for the ordinary binder above referred to, I am able to produce a paper having a "pop" strength of substantially 60, or even higher.

The solvent of the casein which I preferably use, comprises an alkaline mixture of sodium fluoride with calcium hydroxide, and I find that these two ingredients react with the fibers in the pulp and render them water-repellent to a marked degree in the paper or board product. The solvent for the casein, that is to say, the ingredients which render the casein water-soluble, also react with the fibers of the pulp, as for instance, with cellulose pulp and to substantially decrease the water absorptive properties of the fibers and par-

ticularly to impart to the papers made from such pulp these properties of water resistiveness and toughness.

The introduction of my binding material into the beater has the further effect of greatly reducing the number of revolutions through which the beating operation must be carried to produce a thorough and proper mixing of the paper stock or cellulose therewith. In other words, with the use 10 of my improved binding material, the length of time that the stock must be beaten is substantially reduced, thereby correspondingly reducing the cost of the production of the paper or other product.

15 It is possible that sodium carbonate or tri-sodium phosphate or even borax may be substituted for sodium fluoride in the above composition for the production of a paper or board suitable for certain uses but the said materials do not retard the reaction between the casein and the lime as satisfactorily as does the said fluoride.

20 The water-resistiveness of the finished product may also be substantially increased by the addition to the pulp of a relatively small quantity of 25 formaldehyde. In practice, about one ounce of formaldehyde should be used to each 100 pounds of pulp under treatment, but the formaldehyde must be added to the pulp with great care and in small quantities and diluted, since it tends to produce a coagulation of the entire mass under treatment. I preferably dilute the formaldehyde with 30 a small amount of aqua ammonia and warm water, the quantity of ammonia being sufficient to neutralize or nearly neutralize the acid reaction 35 of the formaldehyde. I preferably employ a warm mixture, the water being preferably of a temperature of from 90° to 110° F.

35 In addition to hardening the paper or board and increasing its resistiveness to water or moisture, 40 the formaldehyde also preserves the pulp from deterioration and its incorporation into the pulp is often desirable for this feature also.

45 The formaldehyde thus added to the mixture performs a further function or produces an additional result of rendering the paper more water-proof for it tends to precipitate the casein which is in the fibers and during the web forming step of the paper making process and to firmly bind the fibers together.

50 It not frequently happens that a cellulose pulp is not used in the paper or board making machine for sometime after it has been prepared, and to meet such contingencies, I prefer to also add to the pulp in the beater, and prior to the 55 completion of the beating operation, an additional preservative, such, for instance, as sodium naphthalene sulphonate alpha and to add the same, I preferably dilute it in hot water and add it to the pulp in small quantities. The amount of 60 sodium naphthalene sulphonate alpha should generally not exceed 5% of the weight of the batch of the pulp under treatment.

65 The paper or board made pursuant to my above process produces a water-resistant hard paper product which, upon being folded or creased, tends to crack or break. I have found that I may modify the product in such a way as to make the sheets more flexible and to make 70 them capable of being folded, bent and creased, without breaking, by adding to the batch in the beater a small quantity of a water soluble soap. When soap is added, the final product (paper or cardboard) can be readily folded and creased 75 without substantially decreasing the strength and

water-resistiveness of the paper at the fold or crease.

The addition of soap or soap producing ingredients into the pulp in the beater tends to produce a frothing or foaming of the pulp which is often undesirable. I have found that frothing of the pulp during the beating operation, due to the presence of soap in the pulp, may be greatly reduced by also adding to the pulp a small quantity of light mineral oil to effectively contribute to the water-resisting properties of the final or finished product, to render the paper somewhat more flexible, and to greatly reduce the foaming or bubbling in the beater. The oil may, however, be added to the casein before it is mixed with the lime and fluoride. One pint of such light oil to 100 pounds of casein is sufficient to accomplish these results in most instances.

15 I find that the softening of the final product, (and by "softening" I mean imparting to the product of the property of being readily folded and creased without impairing the water-resistiveness or the strength of the paper) may also be produced with the use of light fatty oils, such as palm oil or olive oil, but to use them I preferably reduce them to a soapy condition by the addition thereto of a suitable alkali and to utilize this soap for its "softening" properties.

20 In describing my invention, I have not referred to any of the fillers which may be employed in the manufacture of paper or board from a cellulose pulp, because the use of these fillers is well known and common in the art. Any of the ordinary filling materials such as asbestos, mineral wool, sodium silicate, clay, portland cement, ground cork and similar fillers used in the various arts in the finished products ordinarily made from cellulose pulp, may be added to the pulp in suitable quantities and at suitable times, without departing from the spirit and 115 scope of my invention.

25 Having thus described my invention, what I claim and desire to protect by Letters Patent of the United States is:

30 1. In the process of making paper and similar cellulose products, the improved method of 120 treating the pulp, which consists in adding to the cellulose fibers in its alkaline liquor in the beater, a binder for the fibers thereof consisting of a proteid containing casein and in quantities from 125 2 to 6 pounds of the proteid of each 100 pounds of the pulp in the beater, lime from 10% to 20% of the weight of the proteid and sodium fluoride from 5% to 8% of the weight of the proteid and continuing the treatment of the pulp in the beater 130 until the mass is homogeneous and the fibers are of the desired degree of fineness.

35 2. In the process of making paper and similar cellulose products, the improved method of 135 treating pulp which consists in beating cellulose pulp in its liquor, and in the presence of a proteid containing casein, in quantity from 2 to 6 pounds of the proteid for each 100 pounds of pulp under treatment, lime, from 10% to 20% of the weight of the proteid and sodium fluoride, from 5% to 140 8% of the weight of the proteid.

40 3. In the process of making paper and similar cellulose products, the improved method of 145 treating pulp, which consists in beating the cellulose into a pulp in its liquor and in the presence of casein, from 2 to 6 pounds of casein for each 100 pounds of pulp under treatment, lime from 10% to 20% of the weight of the casein, sodium fluoride from 5% to 8% of the weight of the casein, and formaldehyde diluted with water and 150

having its acid reaction substantially neutralized with an alkali.

4. In the process of making paper and similar cellulose products, the improved method of treating pulp, which consists in beating the cellulose into a pulp in its liquor and in the presence of casein, from 2 to 6 pounds of casein for each 100 pounds of pulp under treatment, lime from 10% to 20% of the weight of the casein, sodium fluoride from 5% to 8% of the weight of the casein, and formaldehyde diluted with water and having its acid reaction substantially neutralized with aque ammonia. 80

5. In the process of making paper and similar cellulose products, the improved method of treating pulp, which consists in beating the cellulose pulp in its liquor and in the presence of casein, from 2 to 6 pounds for each 100 pounds of pulp under treatment, lime from 10% to 20% of the weight of the casein, sodium fluoride from 5% to 8% of the weight of the casein, a water soluble soap and a nonsaponifiable oil. 85

6. In the process of making paper and similar cellulose products, the improved method of treating pulp, which consists in beating the cellulose pulp in its liquor and in the presence of casein, from 2 to 6 pounds for each 100 pounds of pulp under treatment, lime from 10% to 20% of the weight of the casein, sodium fluoride from 5% to 8% of the weight of the casein, and sodium naphthalene sulphonate alpha dissolved in water and in quantity substantially 5% of the weight of the pulp under treatment. 90

7. In the process of making paper and similar cellulose products, the improved method of treating pulp, which consists in beating the cellulose pulp in its liquor and in the presence of casein, from 2 to 6 pounds for each 100 pounds of pulp under treatment, lime from 10% to 20% of the weight of the casein, sodium fluoride from 5% to 8% of the weight of the casein, and sodium naphthalene sulphonate alpha dissolved in water and in quantity substantially 5% of the weight of the pulp under treatment. 95

weight of the casein, sodium fluoride, from 5% to 8% of the weight of the casein, sodium naphthalene sulphonate alpha dissolved in water and in quantity substantially 5% of the weight of the pulp under treatment, and a small quantity of formaldehyde diluted with water and with aqua ammonia in a quantity sufficient to substantially neutralize the acid reaction of said formaldehyde.

8. In the process of making paper and similar cellulose products, the improved method of treating the pulp, which consists in beating cellulose fibers in the liquor therefor and in the presence of a proteid, lime from 10 to 20% of the weight of said proteid, and sodium fluoride from 5 to 8% of the weight of the proteid. 100

9. In the process of making paper and similar cellulose products, the improved method of treating the pulp, which consists in beating cellulose fibers in the liquor therefor and in the presence of a proteid and a fluoride. 105

10. In the process of making paper and similar cellulose products, the improved method of treating the pulp, which consists in beating cellulose fibers in the liquor therefor and in the presence of casein, lime and a fluoride. 110

11. The method of indurating and waterproofing paper and similar cellulose products, which consists in impregnating the cellulose fibers of which such product is composed, with casein, an alkali which renders said casein soluble in water and a fluoride. 115

12. The method of indurating and waterproofing paper and other fibrous fabrics, which consists in impregnating the fibers of which such fabric is composed with casein, an alkali which renders said casein soluble in water, a fluoride and a small quantity of a softening ingredient. 120

MONE R. ISAACS.

115

40

45

120

50

125

55

130

60

135

65

140

70

145

75

150